

July 13, 1954

C. G. GOETZEL

2,683,305

MOLYBDENUM COATED ARTICLE AND METHOD OF MAKING

Filed July 15, 1949



INVENTOR.  
CLAUSS G. GOETZEL  
BY  
Hammond & Littell  
ATTORNEYS

## UNITED STATES PATENT OFFICE

2,683,305

MOLYBDENUM COATED ARTICLE AND  
METHOD OF MAKINGClaus G. Goetzel, Yonkers, N. Y., assignor to  
Sintercast Corporation of America, New York,  
N. Y., a corporation of New York

Application July 15, 1949, Serial No. 105,035

6 Claims. (Cl. 29—198)

1

This invention relates to protective surfaces for structural components useful under high temperature and corrosive atmosphere conditions and particularly to protective surfaces or casings for the refractory metal molybdenum, the protective surface casings being integrally fused and diffused with the base substance.

Components suitable for use as buckets, blades, valves, nozzles, and the like, in gas or steam turbines, jet engines and devices having similar temperature and atmosphere conditions present problems difficult to solve. Such components must have certain desirable physical characteristics so that they will withstand the stresses involved and yet will not deteriorate under oxidizing or corrosive conditions. The elements must have high hot tensile strength, hot fatigue strength, and high resistance to creep at elevated temperatures.

Molybdenum possesses certain desirable characteristics which make it adaptable for structural materials exposed to high temperatures. Molybdenum in contrast to some other of the refractory metals is not very much heavier than certain of the alloy steels, nickel base alloys or cobalt base alloys, the specific gravity of molybdenum being 11.2. Because of its high fusion and evaporation temperatures, molybdenum has a very high modulus of elasticity which is in the order of 50,000,000 pounds per square inch. This indicates a high resistance to deformation and creep at very high temperatures. Also, the strength of molybdenum is high, particularly if in the wrought condition. For wire and sheet materials, a tensile strength of 90,000 pounds per square inch at 1100° F., and 37,000 pounds per square inch at 2000° F. is attainable.

In order to utilize these desirable physical properties, it is necessary to preserve the fine grain structure of the highly worked molybdenum metal. It also is important in subsequent treatments applied to the metal, not to overheat beyond about 2200° F., because in high purity molybdenum, such will cause excessive recrystallization and grain growth.

Molybdenum is abundantly found in the United States and its mining processes, metallurgy, physical metallurgy and metal working practices have been perfected. Further, the production of molybdenum products by powder metallurgy techniques, and also lately by casting techniques, has been perfected so that large ingots and shapes up to 250 pounds and sizes up to 7" in diameter and 30" in length can now be produced.

One of the biggest difficulties has been that

5 molybdenum is increasingly susceptible to oxidation at temperatures above 1100° F. This is because the reaction of molybdenum with oxygen results in the formation of molybdenum trioxide which becomes highly volatile at temperatures above 1650° F. Because of this, when the metal is exposed to temperatures of 1650° F. and higher, a rapid thermal decomposition will take place and the metal will be destroyed by the attack of oxygen. The attack will progress from the periphery to the core of the exposed body.

10 Because of this problem, it has been recognized that unless a protective atmosphere or vacuum is provided, such as in incandescent lamps or 15 X-ray tubes, access of oxygen to the surface of the molybdenum must be prevented by employing physical or physico-chemical means which will permit retention of the metallic structure of molybdenum up to the temperature limits set 20 by the aforementioned recrystallization and grain growth.

25 Surface protection has been attempted by conventional means such as by enveloping the metal in a stable ceramic, such as Silimanite or alumina, in the form of shells, tubes, etc. Spraying of the ceramic material in the form of a slurry and subsequently baking also was tried as well as slip-casting various washes of ceramic compositions differing in thermal expansivity and 30 cementing properties. Other physical processes have been tried such as the surface deposition of metallic, semi-metallic or metalloidal substances onto molybdenum by such chemical treatments as precipitation or reaction displacement methods 35 from suitable salts, these processes being carried out at ordinary temperatures or elevated temperatures. Electro-deposition, deposition from the vapor phase, or thermal decomposition from certain compounds also have been tried. In the 40 coating processes just mentioned, the surfacing or casing did not achieve lasting results.

45 Molybdenum metal regardless of its comparatively large atomic radius and high heat of reaction due to its high melting point has a high coefficient of diffusion at elevated temperatures and molybdenum for this reason penetrates at an increasingly rapid rate with rising temperature into other high melting metals as well as into alloys or compounds. Stable compounds such as 50 the refractory oxides  $Al_2O_3$ ,  $SiO_2$  or  $MgO$  when brought into contact with molybdenum metal at high temperatures are penetrated by the molybdenum. It can be theorized that place exchange reactions occur so that the molybdenum atoms switch positions with aluminum, silicon, or mag-

nesium in the compounds and that complex compounds of the type containing the elements molybdenum and/or molybdenum oxide com-silicon, oxygen; or molybdenum, magnesium, oxygen are formed. There is a possibility that molybdenum atoms migrate through a grain boundary until they reach exposed surfaces. It also is possible that the stable oxides are locally reduced by the molybdenum and that the resulting molybdenum trioxide because of its very high vapor pressure penetrates through the crystal structure or the boundary regions of the stable compound. In any event, the penetration of the molybdenum and/or molybdenum oxide, compounds result in exposure to erosion and corrosion of the protective stable oxide surfaces.

One of the objects of this invention is the protection of molybdenum by utilizing a surfacing or casing method which provides for the protection (physically, chemically and metallurgically) of the molybdenum base metal, said surfacing or casing method also protecting the molybdenum against deterioration.

In one aspect of the invention, intermediary layers are placed between the molybdenum base and the corrosion resistant surface casing. The proper selection of the intermediate layer will enable formation of intermetallic compounds with the molybdenum, these compounds constituting the necessary barriers respective to diffusion of the molybdenum into the surface casing and the surface metal into the molybdenum base. This is based on the fundamental diffusion laws which hold that diffusion rates are retarded in the presence of compounds so that migration of the molybdenum through a barrier of molybdenum containing intermetallic compounds will be slowed down. If, however, the compound functioning as a diffusion barrier is not of the intermetallic type, such as the system molybdenum-iron or molybdenum-nickel, but is of a non-metallic type, such as a carbide, boride, silicide, etc., either of molybdenum or even better of a foreign metal or non-metal, outward diffusion of molybdenum will be further inhibited.

It is a further object of the invention to produce synthetically, an intermediate layer in such a way as to offer one or, if possible, several successive continuous layers functioning as "moderators" or slow-down agents for the migrating molybdenum atoms, thus providing a casing for a molybdenum base metal which will be stable for long periods of time under high temperature oxidizing atmospheres.

By introducing soft and plastic metal layers, between the non-metallic compound barrier layers, stress concentrations due to differences in expansivity or externally caused stresses, such as centrifugal forces, dynamic loads, etc., are relieved or eliminated.

These and other objects, advantages and features of the invention will become apparent from the following description and drawings.

Figure 1 diagrammatically illustrates one form of the invention.

Figure 2 diagrammatically illustrates another form of the invention.

Figure 3 illustrates one type of apparatus which may be used for coating molybdenum sheet.

Figure 4 represents another type of apparatus which can be used for coating molybdenum sheet.

Figure 5 is an enlarged view of molybdenum sheet showing one manner in which the edges can be covered.

In one form of the invention, an intermediate

layer of an iron-nickel alloy containing between 36% and 50% nickel can be used. The nickel, iron, or similar alloy layer can be produced on the molybdenum base in various manners such as by electro-deposition, spray coating or by the carbonyl process.

The pure metals iron, nickel, or cobalt; binary alloys of iron and nickel, iron and cobalt or nickel and cobalt; ternary alloys of iron, nickel and cobalt can be electro-deposited in a conventional manner in any desired ratio onto the finished molybdenum body. In case of an alloy, the deposit may either be of a homogeneous type, solid solutions for most ratios, or it may be deposited in individual successive layers or zones. The electro-deposit is then diffused and merged with the molybdenum base part by a subsequent heat treatment under protective atmospheres. Due to the comparative stability of electro-deposits, temperatures of a high order and prolonged times are required for the diffusion processes.

The pure metals iron, nickel and cobalt; the binary alloys of iron with nickel, iron with cobalt and nickel with cobalt; and the ternary alloys of iron, nickel and cobalt in any desired proportion can be applied to the molybdenum base by conventional spray methods. For this purpose, the metal or alloy can be employed in wire form or as an alloyed and disintegrated powder. Also, the metals can be deposited in individual layers and their diffusion controlled in the subsequent treatment to give the desired concentration zones for adequate matching of their expansivity with that of the base metal or the ultimate surface material. Due to the history of such spray coatings, which in general employ slightly oxidizing conditions, an intensive reduction and diffusion treatment is required for perfect bonding and merging of the deposit with the molybdenum base metal.

The metals iron, nickel and cobalt; the binary alloys between iron and nickel, iron and cobalt, nickel and cobalt; and the ternary alloys of iron, nickel and cobalt; and also binary, ternary or quaternary alloys of the metals iron, nickel and cobalt, respectively, with molybdenum, the latter preferably in minor proportion, can be deposited on the molybdenum base by the thermal decomposition of the respective metal carbonyls. This method, employing the formation of the simple or multiple carbonyl compounds by the well-known process of combining the metal or alloy in question with carbon monoxide into the liquid compounds with the aid of high pressure (up to 2000 atms.) and a slightly elevated temperature (about 200-400° F.), followed by a decomposition of the complex carbonyl compound at a somewhat higher temperature (about 600-800° F.) and ordinary pressures, is particularly suitable for the purpose of this invention. The deposits obtained, being either in form of a powder or of a sponge or as a coherent solid film or layer depending on the conditions prevailing in the decomposition chamber with the latter type of deposit obtainable when the molybdenum part is suspended directly in the heat zone of the decomposition chamber, are highly reactive and known to result in high rates of diffusion at very low temperatures such as in the range of 1200-1650° F. It is this latter fact which is of particular importance, since it enables diffusion bonding of the layer to the molybdenum at a temperature level which is safely below the one at which any significant changes in grain structure or physical properties could occur.

Thereafter an oxidation proof and corrosion resistant surface casing can be placed on top of the intermediary alloy layers which is described. The preferred manner for deposition of the surface metal is by the vapor phase methods involving either pure metal or a compound of metal that thermally decomposes upon deposition, initiating a metal atom exchange process. In the case of pure metals, chromium, silicon, zirconium, or aluminum, are the most desirable. Although pure chromium as surfacing casing is desirable for reasons of technical simplicity and economy of the process, the oxide of chromium ( $\text{Cr}_2\text{O}_3$ ) formed when exposing the metal to high temperature oxidizing atmospheres lacks some stability from a mechanical standpoint, and tends to mechanically disintegrate and flake and spall off, thus, constantly exposing fresh metal surfaces to the oxidizing atmosphere. This would eventually result in completely wearing through the chromium metal surface. Hence, metals giving more stable oxide films, such as zirconium, silicon, or aluminum are preferred for very high temperature application (above 2000° F.).

If the case formation process employs the previously mentioned mechanism of preferred decomposition of a compound, the halides of chromium, silicon, zirconium, or aluminum, such as chromous chloride, chromous iodide, silicon chloride, zirconium chloride, or aluminum chloride are suitable for the process.

Instead of the pure metals, it may be more advantageous and preferred to employ alloys of chromium with other metals mentioned which tend to form more stable complex oxides. Examples of alloys of chromium with elements to form a more stable oxide, are compounds of chromium with aluminum, with silicon, with zirconium, with aluminum and silicon, with aluminum and zirconium, or with aluminum, silicon and zirconium. In either case, double or triple halides, such as the chlorides, bromides or iodides of chromium plus aluminum, chromium plus silicon, chromium plus zirconium, chromium plus aluminum plus silicon, chromium plus aluminum plus zirconium, or chromium plus aluminum plus silicon plus zirconium, must then be employed.

Reference also may be made to applicant's copending application, Serial No. 94,092, filed May 19, 1949 (now U. S. Patent No. 2,612,442), for details of the various manners of depositing the surface casing on the intermediate layers. The comparatively high degree of surface activity of the carbonyl type deposit is of great advantage in producing integral bonding, fusion and merger between the surface casing metals, alloys or compounds on the one hand and the intermediate layer and the base metal on the other. Thus, low temperatures and short times can be used for the deposition, displacement and atom exchange processes underlying the oxidation proof case formation, which is of great advantage in view of the desirability to prevent heating the molybdenum base metal above its recrystallization temperature.

In another aspect of the invention, the molybdenum base metal part can be carburized and then a soft metal introduced, such as iron, nickel or their alloys, by electroplating, spraying or carbonyl vapor deposition. The carburizing will result in a gradient of carbon concentration. Bonding then can be accomplished by appropriate diffusion treatment prior to application of

the stable oxide surface casing. The bonding treatment subsequent to carburizing can, if necessary, be performed at a temperature above the melting point of the iron, nickel or alloy thereof. This will result in impregnating any pores produced during the carburizing of the molybdenum with the liquid metal or alloy, respectively.

Instead of the formation of carbides, etc., of molybdenum, similar compounds can be formed from other metals or non-metals, such as iron carbide or a complex carbide of iron and silicon, or nickel and silicon, or iron and boron, or nickel and boron. Conventional packs for gas carburizing methods can be used advantageously on iron or some of the other metal or alloy layers which have been deposited previously on or bonded with the molybdenum base metal surfaces. The aforementioned carbonyl vapor process has the advantage of sufficient flexibility to allow the deposition of successive layers of iron, iron carbide, nickel and the like, in any desired sequence and to any desired layer thickness in one operation. By varying the cycle with regard to temperature and time, it is possible to deposit a considerable number of alternate layers of the iron type metal and an alloy rich in iron carbide.

In the case of other barrier compound forming metals to be deposited as intermediate layers, silicon and aluminum are of particular significance since they are also constituents of the complex ultimate surface casing, thus, functioning as diffusion and reaction "moderators" ahead of the reaction process involving the ultimate complex surfacing casing.

Aluminum deposits can be applied, either directly onto the molybdenum, or on an intermediate layer of iron, nickel, or nickel-iron alloy, by dipping the body into the liquid metal, into a suspension in a fused aluminum halide bath, or by placing into an enclosure in a calorizing powder pack. Silicon deposits likewise can be produced directly on the molybdenum, or the intermediate iron, nickel, or nickel-iron alloy layer. Pack siliconizing as well as thermal decomposition of silicon halides are suitable methods for application of silicon deposits. It also is possible to combine the above cited treatments with the aforementioned carburizing treatment, which is particularly advantageous in the case of silicon-carbon combinations which yield the very stable silicon carbide compound, a most effective inhibitor to diffusion of metals.

As previously mentioned, iron, nickel and iron-nickel compounds can be deposited on the molybdenum base to form an intermediate barrier layer. The outer casing is thereafter deposited as described.

Referring to Fig. 1, direct coverage of molybdenum is illustrated, the molybdenum base being indicated at 10 with a Type I layer 11 thereon, said layer consisting of carbon, boron, aluminum, silicon, boron carbide, silicon carbide, and other metals and compounds combined with the molybdenum into complex compounds. Layer 11 is placed on the molybdenum in any of the manners previously described. The next layer 12, a Type II layer, may be of iron, nickel, or iron-nickel alloys as previously mentioned, of a type to diffuse into the compound of the first layer of material 11 or to alloy with molybdenum. The outer case or surfacing material 13, Type III layer, may be chromium, silicon, or aluminum, or binary or ternary alloys thereof, bonding and conversion into stable complex oxide compounds being accomplished by diffusion treatment.

An indirect coverage of molybdenum is seen in Figure 2 wherein the molybdenum body is indicated at 14 having intermediate layers 15 and 16 (Type II) of iron, nickel, iron-nickel alloys, to diffuse or penetrate layer 17 or to alloy with the molybdenum. Layer 17 (Type I) may be carbon, boron, aluminum, silicon, boron carbide, silicon carbide, combined with the molybdenum to form complex compounds. The outer casing 18 (Type III) may be chromium, silicon, aluminum, or 10 binary or ternary alloys thereof.

The various layers may be formed or deposited as follows:

Type I

1. Carburizing:
  - a. gas carburizing
  - b. pack carburizing
2. Aluminizing:
  - a. liquid metal dip
  - b. halide salt bath immersion
  - c. halide gas decomposition
3. Siliconizing:
  - a. pack-impregnation
  - b. halide gas decomposition

Type II

1. Spraying
2. Electroplating
3. Carbonyl process

Type III

1. Pack-impregnation
2. Halide gas decomposition
3. Halide salt bath immersion

As an example of one method of surfacing molybdenum sheet with silicon carbide or boron carbide serving as the intermediate barrier layer against diffusion, reference may be made to Fig. 3 wherein the molybdenum sheet is indicated at 19. The sheet preferably is shot-blasted in order to obtain a proper anchorage. The sheet is fed past a feed hopper 20 containing the carbide grains or a mixture of carbide grains and iron or molybdenum powder. The sheet is passed through a heating furnace 21 having a protective atmosphere, the temperature of said sheet being raised to 1290-1830° F. The sheet is then passed between two carbide rolls 22. In order to cover the other side of the sheet, it can be reversed and again passed through the apparatus.

Another manner in which the carbide can be placed on this sheet is illustrated in Figure 4 wherein the shot-blasted molybdenum sheet 23, is passed through heating furnace 24, said furnace being maintained with a protective atmosphere therein. Said sheet is heated to a temperature between 1290-1830° F. Spray guns 25 can be located on either side of the sheet for spraying hot SiC or B<sub>4</sub>C particles with or without iron or molybdenum powder admixed as a binder.

Various methods can be used to insure that the edge is properly covered. For example, the strip 26 (Fig. 5) can have the carbide surface 27 formed thereon with upstanding portions 28, 29 which can be rolled over the edges to cover the same at 29, 29 to completely protect the sides of the sheet 26. Also, the edges of the sheet could be pointed so that the carbide surface would cover substantially the entire sheet face including the sloping face.

An example of one type of surfaced body is one wherein the molybdenum base is carburized by a gas carburizing process, Mo<sub>2</sub>C being formed. Iron is then deposited on the carburized molybdenum base body by the carbonyl process and

thereafter a silicon-chromium alloy is deposited on the iron layer by a pack-impregnation process.

Another example of the invention is one wherein the molybdenum base has iron deposited thereon by the carbonyl process followed by carburization of the iron layer to form Fe<sub>3</sub>C. The carburization is carried out so that there is a gradient of carbon concentration. Thereafter, another casing of iron is formed by the carbonyl process and a silicon-chromium outer casing integrally merged in a pack-impregnation procedure.

A third example is one wherein the molybdenum base is aluminized by a pack-impregnation deposition procedure. Following this, iron is deposited thereon by a carbonyl process and the iron carburized. Another layer of iron can be deposited by the carbonyl process, and a silicon-chromium-aluminum outer casing then integrally merged with the body by means of a pack-impregnation procedure and heat treatment.

A fourth example is one similar to the aforementioned third example with the exception that a casing of iron is integrally merged with the molybdenum base before deposition of aluminum.

A fifth example is one wherein the molybdenum base is siliconized by a pack-impregnation process and then has iron deposited thereon by means of a carbonyl process. Following this, a silicon-chromium casing is deposited by a pack-impregnation technique and then integrally merged therewith.

A sixth example is one wherein the molybdenum body has iron deposited thereon by means of the carbonyl process followed by siliconizing by pack-impregnation. Iron is then deposited thereon by the carbonyl process and thereafter the iron is carburized by means of pack carburizing. A further coating of iron then is deposited thereon by a carbonyl technique. The outer casing of silicon-chromium then is placed thereon by pack-impregnation and integrally merged with the body.

As a seventh example, the third example can have the coating of iron replaced with a coating of iron-nickel with a nickel content of 36-50%, said iron-nickel being deposited by a carbonyl process.

The eighth example is similar to the aforementioned sixth example, except that an iron-nickel alloy is placed directly on the molybdenum before deposition of silicon thereon.

Pack-impregnation is disclosed in detail in applicant's aforementioned co-pending application Serial No. 94,092 (now U. S. Patent No. 2,612,442). In general, pack-impregnation can be carried out by placing the body in a pack composed of the pulverized material involved and passing a halide gas through the pack at the required high temperature.

It is to be understood that variations may be made in the examples of techniques without departing from the spirit of the invention except as defined in the appended claims.

What is claimed is:

1. In a method of inhibiting the volatilization of molybdenum as molybdenum trioxide resulting from the reaction of a molybdenum-base body with oxygen-containing atmospheres at elevated temperatures, the improvement which comprises providing a coating of at least one intermediate layer of a metal selected from the group consisting of iron, nickel, cobalt and alloys thereof on the exposed surface of said molybdenum-base body, subjecting the thus-coated body to heating in a non-oxidizing atmosphere at

an elevated temperature sufficient to integrally merge said layer to the molybdenum-base body by diffusion so as to form a barrier zone thereon with molybdenum, then surfacing said coated molybdenum-base body with at least one protective layer of metal selected from the group consisting of chromium, silicon, aluminum, zirconium and alloys thereof and bonding said protective surface layer of metal to said intermediate barrier zone layer by diffusion heat treatment, whereby the intermediate barrier zone substantially inhibits the migration of atoms of molybdenum to the surface of the body and of atoms of the surface metal layer into the molybdenum-base body such that the attack of the molybdenum-base body by oxygen-containing atmosphere is greatly inhibited at elevated temperatures of about 1650° F. and higher.

2. In a method of producing components from a molybdenum-base body adapted to withstand corrosion at elevated temperatures and suitable for the production of buckets, blades, valves, nozzles, and the like, in gas turbines, steam turbines, jet engines and other devices employed under comparable temperature and atmospheric conditions, the steps comprising providing a coating of at least one intermediate layer of a metal selected from the group consisting of iron, nickel, cobalt and alloys thereof on the exposed surface of said molybdenum-base body, subjecting the thus-coated body to heating in a non-oxidizing atmosphere at an elevated temperature of at least about 1200° F. to integrally merge said layer by diffusion to the molybdenum-base body so as to form a barrier zone thereon with molybdenum, then surfacing said coated molybdenum-base body with at least one protective layer of metal selected from the group consisting of chromium, silicon, aluminum, zirconium and alloys thereof and bonding said protective surface layer of metal to said intermediate layer by diffusion heat treatment, whereby the intermediate barrier zone substantially inhibits the migration of atoms of molybdenum to the surface of the body and atoms of the surface metal layer into the molybdenum-base body such that the protectively surfaced molybdenum-base body has substantially improved resistance to deterioration and to catastrophic oxidation at elevated temperatures of about 1650° F. and higher.

3. In a method of producing components from a molybdenum-base body adapted to withstand corrosion at elevated temperatures and suitable for the production of buckets, blades, valves, nozzles, and the like, in gas turbines, steam turbines, jet engines and other devices employed under comparable temperature and atmospheric conditions, the steps comprising providing a coating of at least one intermediate layer of a metal selected from the group consisting of iron, nickel, cobalt and alloys thereof on the exposed surface of said molybdenum-base body, subjecting the thus-coated body to heating in a non-oxidizing atmosphere at an elevated temperature of at least about 1200° F. to integrally merge said layer by diffusion to the molybdenum-base body so as to form a barrier zone thereon, then surfacing said coated molybdenum-base body with a protective layer of metal selected from the group consisting of chromium, silicon, aluminum, zirconium and alloys thereof by deposition from a vapor phase containing said metal and bonding said protective surface layer of metal to said intermediate layer by diffusion heat treatment, whereby the intermediate barrier zone sub-

stantially inhibits the migration of atoms of molybdenum to the surface of the body and atoms of the surface metal layer into the molybdenum-base body such that the protectively surfaced molybdenum-base body has substantially improved resistance to deterioration and to catastrophic oxidation at elevated temperatures of about 1650° F. and higher.

4. In a method of producing buckets, blades, valves, nozzles, and the like, for use in gas turbines, steam turbines, jet engines and other devices employed under comparable temperature and atmospheric conditions from a molybdenum-base body, the steps comprising forming a gaseous metal carbonyl phase containing a metal carbonyl selected from the group consisting of iron, nickel and cobalt carbonyl and mixtures thereof, bringing said metal carbonyl phase in contact with said molybdenum-base body, decomposing said gaseous metal carbonyl phase at a temperature of about 600° F. to 800° F. and depositing a coating of at least one intermediate layer of a metal selected from the group consisting of iron, nickel, cobalt and alloys thereof on the exposed surface of said molybdenum-base body, subjecting the thus-coated body to heating in a non-oxidizing atmosphere at an elevated temperature of at least about 1200° F. to integrally merge said layer by diffusion to the molybdenum-base body so as to form a barrier zone thereon with molybdenum, then surfacing said coated molybdenum-base body with a protective layer of metal selected from the group consisting of chromium, silicon, aluminum, zirconium and alloys thereof and bonding said protective surface layer of metal to said intermediate layer by diffusion heat treatment, whereby the intermediate barrier zone substantially inhibits the migration of atoms of molybdenum to the surface and atoms of the surface metal layer into the molybdenum-base body such that the protectively surfaced molybdenum-base body has substantially improved resistance to deterioration and to catastrophic oxidation at elevated temperatures of about 1650° F. and higher.

5. In a method of producing buckets, blades, valves, nozzles, and the like for use in gas turbines, steam turbines, jet engines and other devices employed under comparable temperature and atmospheric conditions from a molybdenum-base body, the steps comprising forming a gaseous metal carbonyl phase containing a metal carbonyl selected from the group consisting of iron, nickel and cobalt carbonyl and mixtures thereof, bringing said metal carbonyl phase in contact with said molybdenum-base body, decomposing said gaseous metal carbonyl phase at a temperature of about 600° F. to 800° F. and depositing a coating of at least one intermediate layer of a metal selected from the group consisting of iron, nickel, cobalt and alloys thereof on the surface of said molybdenum-base body, subjecting the thus-coated body to heating in a non-oxidizing atmosphere at an elevated temperature of about 1200° F. to 1650° F. to integrally merge said layer by diffusion to the molybdenum-base body so as to form a barrier zone thereon with molybdenum, then surfacing said coated molybdenum-base body with a protective layer of metal selected from the group consisting of chromium, silicon, aluminum, zirconium and alloys thereof by deposition from a vapor phase containing said metal and bonding said protective surface layer of metal to said intermediate layer by diffusion heat treatment, whereby the intermediate barrier zone sub-

## 11

stantially inhibits the migration of atoms of molybdenum to the surface and atoms of the surface metal layer into the molybdenum-base body such that the protectively surfaced molybdenum-base body has substantially improved resistance to deterioration and to catastrophic oxidation at elevated temperatures of about 1650° F. and higher.

6. A protectively surfaced molybdenum-base body having substantial resistance to catastrophic oxidation in oxygen-containing atmospheres at elevated temperatures which comprises a molybdenum-base portion, an intermediate layer of a metal selected from the group consisting of iron, nickel, cobalt and alloys thereof covering the exposed surface of said portion, said intermediate layer being merged integrally with said molybdenum-base surface and being characterized by a diffusion barrier zone containing molybdenum, and a surface layer of metal selected from the group consisting of chromium, silicon, aluminum, zirconium and alloys thereof covering said inter-

5

## 12

mediate layer and merged therewith, whereby said body has improved resistance to oxidation at elevated temperatures of about 1650° F. and higher.

References Cited in the file of this patent  
UNITED STATES PATENTS

| Number    | Name        | Date          |
|-----------|-------------|---------------|
| 1,650,979 | Brace       | Nov. 29, 1927 |
| 1,718,563 | Kelley      | June 25, 1929 |
| 1,899,569 | Howe        | Feb. 28, 1933 |
| 2,096,924 | Schwarzkopf | Oct. 26, 1937 |
| 2,109,485 | Ihrig       | Mar. 1, 1938  |
| 2,304,297 | Anton       | Dec. 8, 1942  |
| 2,450,851 | Colbert     | Oct. 5, 1948  |
| 2,450,855 | Colbert     | Oct. 5, 1948  |
| 2,450,856 | Colbert     | Oct. 5, 1948  |
| 2,475,601 | Fink        | July 12, 1949 |
| 2,497,090 | Miller      | Feb. 14, 1950 |